# EUROPEAN PATENT SPECIFICATION

(11) **EP 0 150 240 B1**
(45) Date of publication and mention of the grant of the patent: **03.05.1989**
(21) Application number: 84100878.2
(22) Date of filing: 27.01.1984
(51) Int. Cl.: C22C 1/09, B22D 19/14, B22D 13/04

(54) **Fiber reinforced metal alloy and method for the manufacture thereof**
Faserverstärkte metallische Werkstoffe und Verfahren zu ihrer Herstellung
Matériau métallique renforcé par des fibres et procédé pour sa fabrication

(43) Date of publication of application: 07.08.1985
(73) Proprietor: Chugai Ro Kogyo Co., Ltd., Osaka-shi Osaka-fu (JP); KUBOTA LTD., Naniwa-ku Osaka 556 (JP)
(72) Inventor: Shintaku, Yasuyuki, Sennan-shi Osaka-fu (JP); Hiraishi, Hisashi, Tsuzuki-gun Kyoto-fu (JP)
(74) Representative: Glawe, Delfs, Moll & Partner

(56) References cited:
- EP-A- 0 094 970
- WO-A-83/02782
- FR-A- 1 187 139
- FR-A- 2 133 852
- "Modern composite materials", 1968, edited by Lawrence J. Broutman et al., pages 412-418, Addison-Wesley Publishing Company, Reading, Massachusetts, USA;

## Description

The present invention relates to a structural element in the form of a hollow cylindrical element in the form of a hollow cylindrical body, especially a roll, made of fibre reinforced metal alloy and to a method for manufacturing such a structural element.

Hitherto, various types of fibre reinforced metal alloys (FRM) comprising a metal matrix and reinforcement fibres have been proposed. These fibre reinforced metal alloys are composite material wherein the metal matrix comprised, for example, aluminium or titanium and the fibre reinforcement comprises, for example, carbon fibres, silica carbide fibres, boron fibres or alumina fibres. Both the heat resistance and the heat insulating property of any one of these fibre reinforced metal alloys are not so high and, accordingly, they are not suited for use as a material for component parts operable in the high temperature environment, such as, for example, conveyor rolls installed inside a heating furnace for the transportation of materials to be heat-treated and those for the transportation of hot rolled strips.

A structural element of the abovementioned kind and a method for manufacturing such a structural element has been known from e.g. FR-A-2 133 852.

It is the object of the invention to provide a structural element made of fibre reinforced metal alloys which can be used as a material for structural components installed inside a furnace.

This object of the invention is solved by a structural element in the hollow cylindrical body, especially a roll, made of fibre reinforced metal alloy, wherein an annular layer of reinforcing fibre material is embedded in the wall of the structural element such that the metal alloy completely fills the interstices between the fibres of the web, said layer having a defined radial thickness smaller than the wall thickness of the structural member, with layers of metal alloy without reinforcing fibres being provided radially inwardly and outwardly of said layer of fibres.

The method according to the invention comprises the steps of:
positioning an annular layer of reinforcing fibre material within a centrifugal casting mold in spaced relationship from the inner surface of said mold;
pouring a melt of metal alloy into the casting mold; and
rotating the casting mold in one direction so as to permit the melt to flow into the interstices of the layer of fibre material and through said layer into the space between the layer and the inner surface of the casting mold.

These and other objects and features of the present invention will become apparent from the following description taken in conjunction with a preferred embodiment thereof with reference to the accompanying drawings, in which:
Fig. 1 is a longitudinal sectional view showing schematically a centrifugal casting mold according to a first preferred embodiment of the present invention;
Fig. 2 is a cross sectional view taken along the line II-II shown in Fig. 1;
Fig. 3 is a cross sectional view, on an enlarged scale, of a roll manufactured by the use of the casting mold shown in Fig. 1;
Fig. 4 is a cross sectional view, on a further enlarged scale, showing a portion of the roll shown in Fig. 3;
Fig. 5 is a view similar to Fig. 2, showing the centrifugal casting mold according to another preferred embodiment of the present invention;
Fig. 6 is an end view, on an enlarged scale, of one of the support rings used in the casting mold shown in Fig. 5; and
Fig. 7 is a graph showing the temperature distribution in the roll manufactured according to the present invention and the conventional roll.

### DETAILED DESCRIPTION OF THE EMBODIMENTS

Before the description of the present invention proceeds, it is to be noted that like parts are designated by like reference numerals throughout the accompanying drawings. It is also to be noted that, in describing a fiber reinforced metal alloy of the present invention, reference will be made for the sake of brevity to a roll manufactured according to a centrifugal casting method and having a layer of fiber reinforced metal alloy embedded in the roll.

Referring first to Figs. 1 to 4, there is schematically shown a centrifugal casting mold 1 of any known construction. The casting mold 1 is of a generally cylindrical configuration open at both ends thereof and has a centrally perforated end plate 2a or 2b used to close each open end of the casting mold 1. For manufacturing a cylindrical roll, shown by 8 in Fig. 3, having its exterior surface region embedded with a layer of fiber reinforced metal alloy according to the present invention, an interwoven tube 4 of reinforcement fibers, i.e., a fibrous reinforcement formed by interweaving reinforcement fibers so as to present a generally tubular configuration, is positioned coaxially within the casting mold 1 with its opposite ends held in abutment with support rings 3a and 3b one for each end of the interwoven tube 4. For avoiding any possible contact of a substantially intermediate portion of the interwoven tube 4 with the inner peripheral surface of the casting mold 1 during the casting operation, a plurality of ring-shaped spacers 5 are mounted exteriorly on the interwoven tube 4 and arranged in equally spaced relation to each other in a direction lengthwise of the casting mold 1. It is to be noted that, instead of the use of the plurality of ring-shaped spacers 5, a single coil of wire may be used as a spacer for the intended purpose.

Preferably, the reinforcement fibers used to form the interwoven tube 4 are comprised of three-element type fibers containing alumina (AI,0,₃), boron oxide (B₂0₃) and silica (Si0₂) in respective quantities of 62 wt%, 14 wt% and 24 wt%.

The casting of the roll 8 is carried out by pouring a melt of 25Cr-20Ni metal alloy (C: 0.41 wt%, Si: 1.18 wt%, Ni: 20.28 wt%, Mn: 1.02 wt%, P: 0.015 wt%, S: 0.011 wt%, Cr: 24.41 wt%, and Mo: 0.05 wt%) into the casting mold 1 through the central opening 6a in the end plate 2a and then through the central opening 6b in the support ring 3a with the interwoven tube 4 supported therein in the manner described above, and then rotating the casting mold 1 in one direction to allow the melt to be radially outwardly forced to adhere to the inner peripheral surface of the casting mold 1 under the influence of a centrifugal force. During the casting so effected, the melt is forced to flow towards the inner peripheral surface of the casting mold 1 through not only the meshes 4a (Fig. 4) defined in the interwoven tube 4, but also the interstices among the reinforcement fibers forming the interwoven tube 4 and then into a clearance formed by the spacers 5 between the casting mold 1 and the interwoven tube 4. In practice, the amount of the melt poured into the casting mold 1 is so selected that the interwoven tube 4 can be substantially completely embedded in an annular wall of the resultant roll 8 in a manner as shown in Fig. 3.

After the solidification of the melt within the casting mold, the resultant roll 8 is removed out of the casting mold 1. As best shown in Fig. 4, the resultant roll 8 has a layer A of the reinforcement fibers initially defined by the interwoven tube 4 and embedded therein at a location spaced radially inwardly from the outer peripheral surface thereof. To complete the manufacture of the roll 8 having its outer surface region covered substantially by the reinforcement fiber layer A, the roll 8 so cast is subsequently subjected to any known grinding process to remove a surface portion 7 of the roll 8 to make the reinforcement fiber layer A exposed to the outside. However, depending on the particular application in which the roll is used, the removal by grinding of the surface portion 7 may not be always necessary.

It is to be noted that the number of the fibrous reinforcements, shown as the interwoven tube in the illustrated embodiment, may not be always limited to one such as shown, but may be two or more. Where the fibrous reinforcements are laminated, i.e., where two or more interwoven tubes are employed one inside the other in laminated relation, it may happen that the melt of metal alloy will not reach the inner peripheral surface of the casting mold 1 during the centrifugal casting operation. In such case, instead of the use of the spacers 5, a spacer layer of metal having a low melting point such as, for example, AI or Zn within ±15% of the lattice constant of Fe may be centrifugally formed in adherence to the inner peripheral surface of the casting mold 1 prior to the melt of the previously described metal alloy being poured into the mold 1. Where this technique is employed, the aforesaid spacer layer are, when the melt is poured into the casting mold 1 after the spacer layer has been solidified, melted by the heat evolved by the melt and is subsequently dispersed to mix with the melt to ultimately present a diffused solid solution.

It is also to be noted that where the number of the interwoven tubes is two or more, or where the single interwoven tube has so great a wall thickness that the poured melt of the metal alloy will be hard to flow radially outwardly through the interwoven during the centrifugal casting operation even though the above described alternative technique is employed, the interwoven tube may be formed with at least one through-hole at a portion adjacent the central opening 6a so that the melt poured into the casting mold 1 through the central opening 6a can also flow through the through-hole into the clearance between the casting mold and the interwoven tube 4 during the casting operation.

It is further to be noted that, where the reinforcement fibers used are of a nature easy to melt in contact with the melt of metal alloy, the interwoven tube may have a heat resistant coating applied thereto to avoid any possible melt of the reinforcement fibers.

While according to the foregoing embodiment the layer of the reinforcement fibers embedded in the roll is exposed to the outside by grinding the outer surface portion of the roll, which grinding has been necessitated because of the marks left on the outer surface of the roll by the spacer rings 5, the concept of the present invention can equally be applicable to the manufacture of the roll having the reinforcement fiber layer embedded therein at a location substantially intermediately of the wall thickness thereof. This will now be described with particular reference to Figs. 5 and 6.

As best shown in Fig. 5, instead of the spacer rings 5 employed in the foregoing embodiment, outer and inner perforated SUS pipes 9a and 9b, one inside the other, are employed for the support of the interwoven tube 4. In addition, each of the support rings 3a and 3b employed in the embodiment shown in Figs. 5 and 6 is of an outer diameter substantially equal to the inner diameter of the casting mold 1 and has a plurality of spacer projections 10 protruding radially outwardly therefrom and circumferentially equally spaced from each other. Each of the support rings 3a and 3b is formed with outer and inner circular grooves 11a and 11b on one surface thereof in coaxial relation to the axial of rotation of the casting mold 1. The interwoven tube 5 is, after having been inserted into an annular clearance defined between the outer and inner perforated SUS pipes 9a and 9b, supported within the casting mold 1 by the SUS pipes 9a and 9b having their opposite ends received in the respective outer and inner circular grooves 11a and 11b in the associated support rings 3a and 3b as best shown in Fig. 5. It will readily be seen that, because of the particular configuration of each of the support rings 3a and 3b as shown in Fig. 6, the melt of the metal alloy poured into the casting mold 1 through the central opening 6a can flow not only into the inside of the inner SUS pipe 9b through the central opening 6b, but also into the clearance between the outer SUS pipe 9a and the inner peripheral surface of the casting mold 1 through arcuate passages each extending between the adjacent two radially outward projections 10.

During the actual casting operation with the casting mold 1 rotated in one direction about the longitudinal axis thereof, the melt of the 25Cr-20Ni metal alloy poured into the casting mold 1 through the central opening 6a flows on the space 12 between the end plate 3a and the support ring 3a first into the clearance between the outer SUS pipe 9a and the casting mold 1 through the arcuate passages and then into the inside of the inner SUS pipe 9b through the central opening 6b in the support ring 3a. The melt entering the inside of the inner SUS pipe 9b is, during the continued rotation of the casting mold 1, forced under the influence of the centrifugal force to flow into the clearance between the outer and inner pipes 9a and 9b through the perforations in the inner pipe 9b and, substantially at the same time, the outer and inner pipes 9a and 9b are fused in contact with the elevated temperature of the poured melt.

The roll manufactured according to the second preferred embodiment has the reinforcement fiber layer A embedded intermediately of the wall thickness thereof substantially as shown in Fig. 4. It has been found that when the roll cast at 1,600°C by the application of a centrifugal force of 58G in accordance with the second preferred embodiment of the present invention and having a wall thickness of 30mm was tested, it exhibited a temperature distribution as shown by the broken line in Fig. 7. For the purpose of comparison, the temperature distribution exhibited by the conventional roll, 30mm in wall thickness, of the same material as the roll according to the present invention, but having no reinforcement fiber layer is also shown by the solid line in the graph of Fig. 7. In the graph of Fig. 7, the values "0" and "30" of the wall thickness represent the inner and outer peripheral surfaces of the roll. These temperature distributions were obtained by exposing the inner and outer peripheral surfaces of the roll according to the invention and the conventional roll to the atmospheres of 350°C and 1,300°C, respectively.

Although the present invention has fully been described in connection with the preferred embodiment thereof, it is to be noted that various changes and modifications are apparent to those skilled in the art. Accordingly, such changes and modifications are to be understood as included within the scope of the present invention as defined by the appended claims, unless they depart therefrom.

## Claims

1. A structural element in the form of a hollow cylindrical body, especially a roll, made of fibre reinforced metal alloy, wherein an annular layer (4) of reinforcing fibre material is embedded in the wall of the structural element such that the metal alloy completely fills the interstices between the fibres of the web, said layer having a defined radial thickness smaller than the wall thickness of the structural member, with layers (8, 7) of metal alloy without reinforcing fibres being provided radially inwardly and outwardly of said layer (4) of fibres.

2. The structural element as claimed in claim 1, wherein the fibre reinforcing material is of three-element fibres of alumina, boron oxide and silica.

3. The structural element as claimed in claim 1, wherein said fibre reinforcing material is an interwoven or intermingled element of inorganic fibres each containing alumina, boron oxide and silica in a predetermined mixing ratio.

4. A method for manufacturing a structural element as claimed in claim 1, comprising the steps of:
positioning an annular layer of reinforcing fibre material within a centrifugal casting mold in spaced relationship from the inner surface of said mold;
pouring a melt of metal alloy into the casting mold; and
rotating the casting mold in one direction so as to permit the melt to flow into the interstices of the layer of fibre material and through said layer into the space between the layer and the inner surface of the casting mold.

## Patentansprüche

1. Bauelement in Form eines hohlzylinderförmigen Körpers, insbesondere einer Rolle, das aus einer faserverstärkten Metallegierung hergestellt ist, in dem eine ringförmige Schicht (4) aus verstärkendem Fasermaterial so in der Wand des Bauelementes eingebettet ist, daß die Metallegierung die Lücken zwischen den Gewebefasern vollständig ausfüllt, wobei die Schicht eine festgelegte radiale Dicke hat, die kleiner als die Wanddicke des Bauelementes ist, mit Schichten (8, 7) einer Metallegierung ohne verstärkenden Fasern, die von der Faserschicht (4) radial nach innen und außen vorgesehen sind.

2. Bauelement nach Anspruch 1, in dem das faserverstärkende Material aus Fasern der drei Bestandteile Aluminiumoxid, Bortrioxid und Siliziumdioxid besteht.

3. Bauelement nach Anspruch 1, in dem das faserverstärkende Material ein verflochtenes oder vermischtes Element aus anorganischen Fasern ist, die jeweils Aluminiumoxid, Bortrioxid und Siliziumdioxid in einem vorbestimmten Mischverhältnis enthalten.

4. Verfahren zur Herstellung eines Bauelementes nach Anspruch 1, mit den Schritten:
Anordnen einer ringförmigen Schicht aus verstärkendem Fasermaterial innerhalb einer Schleudergußkokille in einem Abstand von der Innenfläche dieser Form;
Gießen einer Schmelze aus einer Metallegierung in die Gießform; und
Rotieren der Gießform in eine Richtung, um zu ermöglichen, daß die Schmelze in die Lücken der Schicht aus Fasermaterial und durch die Schicht hindurch in den Raum zwischen der Schicht und der Innenfläche der Gießform fließt.

## Revendications

1. Elément mécaniquement résistant sous forme d'un corps cylindrique creux, notamment d'un rouleau, formé d'un alliage métallique armé de fibres, dans lequel une couche annulaire (4) d'un matériau à base de fibres d'armature est enrobé dans la paroi de l'élément mécaniquement résistant d'une manière telle que l'alliage métallique remplit totalement les interstices délimités entre les fibres de la nappe, la couche ayant une épaisseur radiale déterminée qui est inférieure à l'épaisseur de paroi de l'organe mécaniquement résistant, des couches (8, 7) d'alliage métallique sans fibres d'armature étant disposées radialement à l'intérieur et à l'extérieur de la couche (4) de fibres.

2. Elément mécaniquement résistant selon la revendication 1, dans lequel le matériau d'armature à base de fibres est formé de fibres à trois constituants contenant de l'alumine, de l'oxyde de bore et de la silice.

3. Elément mécaniquement résistant selon la revendication 1, dans lequel le matériau d'armature à base de fibres est un élément tissé ou imbriqué de fibres minérales contenant chacune de l'alumine, de l'oxyde de bore et de la silice dans un rapport prédéterminé de mélange.

4. Procédé de fabrication d'un élément mécaniquement résistant selon la revendication 1, comprenant les étapes suivantes:
la disposition d'une couche annulaire d'un matériau à base de fibres d'armature dans un moule de coulée centrifuge, à distance de la surface interne du moule,
la coulée d'un alliage métallique fondu dans le moule de coulée, et
l'entraînement en rotation du moule de coulée dans un sens tel qu'il permet à la matière fondue de s'écouler dans les interstices de la couche du matériau à base de fibres et, à travers cette couche, dans l'espace compris entre la couche et la surface interne du moule de coulée.
